# EUROPEAN PATENT SPECIFICATION

(11) **EP 1 886 192 B1**
(45) Date of publication and mention of the grant of the patent: **18.07.2012**
(21) Application number: 06752018.9
(22) Date of filing: 27.04.2006
(51) Int. Cl.: G03G 7/00

(54) **ELECTROPHOTOGRAPHIC MEDIUM COMPOSITION**
ELEKTROFOTOGRAPHISCHE MEDIUM-ZUSAMMENSETZUNG
COMPOSITION D' UN MILIEU ELECTROPHOTOGRAPHIQUE

(30) Priority: 05.05.2005 US 122543
(43) Date of publication of application: 13.02.2008
(73) Proprietor: HEWLETT-PACKARD DEVELOPMENT COMPANY, L.P., Houston TX 77070 (US)
(72) Inventor: ZHOU, Xiao-Qi, San Diego, California 92127-1899 (US); UNDERWOOD, Lisa, Boise, Idaho 83714-0021 (US); MCMANUS, Richard, San Diego, California 97127-1899 (US)
(74) Representative: Engelhard, Markus
(86) International application number: PCT/US2006/016652
(87) International publication number: WO 2006/121680

(56) References cited:
- EP-A- 0 442 567
- EP-A- 0 880 079
- US-A1- 2004 043 240
- Search result for methods of measuring surface resistivity and volume resistivity on http://global.ihs.com.
- article 'International Standard IEC 93'

## Description

### BACKGROUND

The present disclosure relates generally to electrophotographic printing medium compositions, and more particularly to an electrophotographic medium composition including a friction-controlling agent and a charge controlling agent.

Electrophotographic printing involves a device that has a media transportation system. Generally, a single sheet of media is picked up from a storage tray and then delivered to a photoreceptor/transfer belt and fuser to complete an imaging procedure. Advanced color electrophotographic printing devices are generally equipped with different color toner cartridges and a duplexer, which makes it possible to duplex images on both sides of a single sheet. The incorporation of a duplexer may, in some instances, involve more complex media passes. The transportation system inside such a printing device may include a higher possibility for media "jam."

Media "jam" includes a variety of potential problems that may result during media transportation. The "no pick" jam may result when a pick-up roller or a vacuum belt of the device fails to move a sheet from the media tray. "Multiple-pick up" jam may result when more than one sheet is picked up from the storage tray at one time. "Skewing jam" may result from media misalignment in the media pass. Input-tray jam, output-tray jam, registration jam, belt jam, or fuser jam may result when problems arise in the particular location (e.g. the input-tray) in the device. Each of the jams may, in some instances, create poor printing quality, shut-down of the printing device, and/or potential damage of the device. The previously described "jams" may, in some instances, be a result of the design of the media pass, the material choice of the media, the printing parameters, the environmental or media storage parameters, and/or combinations thereof.

Further, coated papers used to create superior image effects in color electrophotographic printing may, in some cases, be more problematic to achieve good running ability or sheet-feeding (i.e. less paper jams) during high speed color electrophotographic printing.

US 2004/0043240 discloses an electrophotographic image receiving sheet with a toner image receiving later containing a release agent and formed on a support sheet for use in a fixing belt type electrophotography.

As such, it would be desirable to provide an electrophotographic medium composition that provides sheet running ability such that jams in the device are substantially prevented or lessened.

### SUMMARY

An electrophotographic medium composition is disclosed. The composition includes a friction-controlling agent and an ionic conduction aid mixed together.

### BRIEF DESCRIPTION OF THE DRAWINGS

Objects, features and advantages will become apparent by reference to the following detailed description and drawings, in which like reference numerals correspond to similar, though not necessarily identical components. For the sake of brevity, reference numerals having a previously described function may not necessarily be described in connection with subsequent drawings in which they appear.
FIG. 1 is a schematic view of an embodiment of a system for electrophotographic printing; and
FIG. 2 is a schematic view of an alternate embodiment of a system for electrophotographic printing.

### DETAILED DESCRIPTION

Embodiment(s) of the electrophotographic printing medium composition are suitable for establishment as a coating on a substrate. The coated substrate may be advantageously used in many applications, one example of which is high-speed color electrophotographic printing. Without being bound to any theory, it is believed that friction control agent(s), in combination with electrostatic charge control and base stock stiffness control, provide a printing media with good running ability in high-speed electrophotographic printing devices over a wide range of environmental conditions.

Referring now to Fig. 1, an embodiment of a system 10 for electrophotographic printing is shown. The system 10 includes an embodiment of the electrophotographic printing medium composition 12 established on opposed sides 14, 16 of substrate 18.

In an embodiment, the substrate 18 is paper. The paper may be made of a fabric stock having a weight ranging from about 60 gram/m² (gsm) to about 300 gsm. In a non-limitative example, the weight ranges from about 70 gsm to about 200 gsm.

The paper substrate 18 may also include any suitable wood or non-wood pulp 13. Non-limitative examples of suitable pulps 13 include groundwood pulp, sulfite pulp, chemically ground pulp, refiner ground pulp, thermomechanical pulp, and/or mixtures thereof. Fillers 15 may also be incorporated into the pulp 13, for example, to substantially control physical properties of the final coated paper. Examples of the fillers 15 include, but are not limited to ground calcium carbonate, precipitated calcium carbonate, titanium dioxide, kaolin, clay, silicates, and/or mixtures thereof. It is to be understood that any desirable amount of filler 15 may be used. In one embodiment, the amount of filler 15 ranges from about 0 wt.% to about 20 wt.% of the substrate 18, and in another embodiment, the amount of filler 15 ranges from about 5 wt.% to about 15 wt.% of the substrate 18.

In preparation of the substrate 18 (e.g. paper stock), internal and surface sizing may be desired. This process may advantageously improve internal bond strength of the substrate 18 fibers, and may also advantageously control the resistance of the coated substrate 18 to wetting, penetration, and absorption of aqueous liquids (a non-limitative example of which includes moisture vapor that may contribute to multiple pick-up jams in high humidity conditions). Internal sizing may be accomplished by adding a sizing agent 17 to the substrate 18 in wet end. Non-limitative examples of suitable sizing agents 17 include rosin-based sizing agent(s), wax-based sizing agent(s), cellulose-reactive sizing agent(s) and other synthetic sizing agent(s), and/or mixtures thereof. It is to be understood that the type and amount of surface sizing agent(s) may substantially improve moisture resistance and may alter the stiffness of the base paper stock.

Surface sizing (i.e. apply sizing agent to the formatted paper roll) may be accomplished by film size press, pond size press and other surface techniques.

The stiffness of the paper stock 18 may be related, at least in part, to the paper thickness. It is to be understood that with substantially the same pulp and filler composition, the thinner the paper caliper is, the lower the paper stiffness will be. In order to achieve enhanced running ability, the stiffness of the paper stock 18, or its flexural rigidity may be controlled, in part because the stiffness of the final system 10 may be dependant upon the stiffness of paper stock 18. The stiffness may be determined, at least in part, by the physical properties and composition of fibers in the pulp 13 and the percentage of fibers to fillers 15. A method such as TAPPI T489OM-92, using a Taber-type stiffness tester, may be used to determine the stiffness of the paper stock 18 and the system 10.

A low jam rate (less than about 1 jam for every 1000 running sheets) in high-speed duplex printing is obtained with a stiffness of the system 10 ranging from about 1 Taber stiffness units (gram centimeter) to about 25 Taber stiffness units in the paper machine direction, and ranging from about 1 Taber stiffness units and about 15 Taber stiffness units in the paper cross machine direction. In another embodiment, the system 10 stiffness ranges from about 2 Taber stiffness units to about 18 Taber stiffness units in the paper machine direction, and from about 1.5 Taber stiffness units to about 10 Taber stiffness units in the paper cross machine direction.

Generally, extreme (high or low) temperature and humidity conditions may contribute to paper jams in printing devices. For example, the color electrophotographic printers running at 10°C and 15% relative humidity and running at 30°C and 80% relative humidity generally show higher jam rates than those running at conventional conditions of 23°C and 50% relative humidity. Without being bound to any theory, it is believed that in the case of low temperature and low relative humidity conditions, the electrostatic charge will build up excessively on the media surface. This electrostatic force may stick two or more paper sheets together to initialize the multi-pick jam. Lower electrical surface and volume resistivity values may advantageously assist in rapid release of the electrostatic charges. However, lower resistivity values may, in some instances, result in a problem with the efficiency of toner transfer, which may lower color density of the printed image.

As such, it has been found that an optimized electrical surface and volume resistivity are desirable. In an of environment of 23°C and 50% humidity, the surface resistivity ranges from 1.0x10⁹ to 8.0x10⁹ OHM/square. In this same environment, the volume resistivity is from 1.0x10⁹ to 5.0x10¹⁰ OHM cm. In an alternate embodiment where the temperature and humidity is lower than 15°C and 10%, respectively, the surface resistivity ranges from about 5.0x10¹² to about 1.0x10¹⁵ OHM/square, and alternately from about 7.0x10¹² to 1.0x10¹⁴ OHM/square; while the volume resistivity ranges from about 1.0x10¹³ to about 1.0x10¹⁵ OHM cm, and alternately from about 5.0x10¹³ to about 5.0x10¹⁴ OHM cm. Typical paper stocks and surface coating formulations generally have higher electrical resistivity than the values according to the embodiment(s) herein.

The electrophotographic medium composition 12 includes a friction controlling agent and an ionic conduction aid, which make up an image-receiving layer 22. It is to be understood that any suitable ionic conduction aid may be used. In an embodiment, the ionic conduction aid is an inorganic electrolyte or an organic electrolyte. It is to be understood that the electrolytes may advantageously assist in controlling the electrical resistivity of the composition 12 and of the system 10. Non-limitative examples of suitable electrolytes include sodium chloride, potassium chloride, sodium sulfate, potassium sulfate, quaternary ammonium salts, polymeric electrolytes, sodium salts of polystyrene sulfonates, ammonium salts of polystyrene sulfonates, sodium salts of polyacrylates, ammonium salts of polyacrylates, sodium salts of polymethacrylates, ammonium salts of polymethacrylates, sodium salts of polyvinyl sulfonates, ammonium salts of polyvinyl sulfonates, sodium salts of polyvinyl phosphates, ammonium salts of polyvinyl phosphates, and/or combinations thereof.

In the high temperature and high relative humidity conditions (such as 30°C and 80% relative humidity), moisture enters the gaps between sheets in a media stack and is absorbed either inside coating layer(s) and base stock, or on the surface of the outermost layer of the coated paper. Due, at least in part, to the difference in the equilibrium of the water pressure between the surface and the air, the sheets may adhere together. To substantially control the moisture level on the media surface and to reduce surface tension, the composition 12 (e.g. image-receiving layer 22) also includes a friction-controlling agent as well as a charge control agent (i.e. the previously mentioned ionic conduction aid). The friction-controlling agent may be in a physical form of polymeric emulsions, polymer dispersions, or combinations thereof. In another embodiment, the friction-controlling agent may be in a physical form of polymeric powders. Non-limitative examples of the friction-controlling agent include carnauba wax, montan wax, paraffin wax, microcrystalline waxes from the distillation of crude oil, synthetic polymers and/or combinations thereof.

Examples of synthetic polymers include, but are not limited to those having a polyolefin backbone structure, such as, for example high density polyethylene, low density polyethylene, polypropylene, and polybutene. Other examples of synthetic polymers include polymeric hydrohalocarbon compounds and polymeric hydrofluoro compounds such as polytetrafluoroethylene.

Aside from the friction-controlling agent and charge control agent (ionic conducting agent) described above, the image-receiving layer 22 may contain other chemical components such as inorganic pigments, polymeric binders, and special functional coating additives.

Inorganic pigments include particulates in a powder or slurry form. Non-limitative examples of such materials include titanium dioxide, hydrated alumina, calcium carbonate, barium sulfate, silica, clay, alumino silicates, alumina, boehmite, pseudoboehmite, zinc oxide, and combinations thereof.

Polymeric binder generally refers to a polymer composition used to provide adhesion between the inorganic particles and other components within the image-receiving layer 22. Binders may also provide adhesion between the image-receiving layer 22 and other established layers (such as base coating layer 20 as shown in Fig. 2). In an embodiment, the binders may be a water soluble polymer or water dispersible polymeric latex. Non-limitative examples of suitable binders include styrene butadiene coplymer, polyacrylates, polyvinylacetates, polyacrylic acids, polyesters, polyvinyl alcohol, polystyrene, polymethacrylates, polyacrylic esters, polymethacrylic esters, polyurethanes, copolymers thereof, and combinations thereof.

It is to be understood that when sheet stiffness and the sheet edge quality resulting from sheet converting processing is in the range of the embodiment(s) herein, the sheet running ability may be characterized by the coefficient of friction (COF) of sheet to sheet, and sheet to rubber (if a rubber pick up roller is used for paper pick-up). The COF is an integrated parameter indicating the chemical and physical properties of the media, examples of which include, but are not limited to surface polarity, surface smoothness, air permeability, moisture level of the media. The sheet-to-sheet static COF in 23°C and 50% humidity ranges from about 0.30 to about 0.55, and alternately from about 0.35 to about 0.50, and the sheet-to-sheet kinetic COF in 23°C and 50% humidity ranges from about 0.15 to about 0.50, and alternately from about 0.20 to about 0.45. Without being bound to any theory, it is believed that too high or too low (i.e. outside of the ranges of the embodiment(s) herein) of a COF may, in some instances, cause either multiple jams or "no pick" jams.

The addition of the friction-controlling agent in the image-receiving layer 22 may advantageously assist in maintaining the COF of the system 10 in the desired embodiment range. In a non-limitative example, a non-polar hydrocarbon synthetic polymer emulsion or dispersion, such as high density or low density polyethylene is used. Suitable examples of polyethylenes include MICHEM Emulsion, MICHEM Lube, and MICHEM Shield, all of which are commercially available from Michelman Inc. located in Cincinnati, Ohio. The friction-controlling agents may act as lubricants, anti-slipping agents, and water resistant agents so that value of COF is controlled in the optimum range and the variation of COF value with environmental changes may be substantially advantageously minimized. In this embodiment, the friction-controlling agent is in the form of an emulsion or dispersion with a mean particle diameter ranging from about 0.1 microns to about 1 micron, and in another embodiment ranging from about 0.3 microns to about 0.5 microns. In this example embodiment, the amount of the friction-controlling agent in the image-receiving layer 22 ranges between about 0.2 parts by weight and about 2 parts by weight based on 100 parts of dry weight of the pigment in the layer 22.

In another example embodiment, the friction-controlling agent is a synthetic polymer with a high molecular weight and a solid micro-particle physical form, such as, for example high density polyethylene powder. In this example, the particle size of the friction-controlling agent ranges between about 1 microns and about 20 microns, and alternately between about 5 microns and about 10 microns. In a particular example using polyolefins, the friction-controlling particles are hydrocarbon backbone polymers with an average molecular weight ranging from about 300,000 to about 600,000.

In an embodiment, the amount of friction controlling agent in the image-receiving layer 22 ranges from about 0.5 parts by weight to about 5 parts by weight, and alternately from about 0.7 parts by weight to about 2.0 parts by weight based on 100 parts by weight of dry inorganic pigments.

It is to be understood that the friction-controlling agent (for example, in its powder form) may be selected, at least in part, based on its mechanical properties. In an embodiment, the modulus of elasticity (as measured by the method ASTM D790) may range between about 180 MPa and about 300 MPa, while Shore hardness may range between about 40 and about 60 (as measured by the ASTM D 2240 method). Further, the melting point of the friction-controlling agent generally ranges between about 50°C and about 150°C. In an example embodiment, the melting point ranges between about 90°C and about 130°C.

Referring now to Fig. 2, the system 10 may optionally include a base coating layer 20 established between the image-receiving layer 22 and the side(s) 14, 16 of the substrate 18 upon which the image-receiving layer 22 is established. As such, the composition 12', as shown in Fig. 2, includes the image-receiving layer 22 and the base coating layer 20. In an embodiment, the base coating layer 20 includes an ionic conduction aid, such as, for example, the inorganic and organic electrolytes described hereinabove. The base coating 20 may also include polymeric binders and inorganic pigments, such as those described herein.

Still further, small amounts of coating additives may be present in either or both of the coating 20 and the image-receiving layer 22. Such additives include, but are not limited to dyes to control paper color, optical brighteners, surfactants, rheological modifiers, cross-linking agents, defoamers, and/or dispersing agents, and or combinations thereof.

In an embodiment of the method of making a system 10, the image-receiving layer(s) 22 are established on one or both of the opposed sides 14, 16 of the substrate 12. In an alternate embodiment, the base coating layer(s) 20 are established on one or both of the opposed sides 14, 16 of the substrate 18, and the image-receiving layers 22 are established on each of the coating layers 20. It is to be understood that the optional coating layers 20 and the image-receiving layers 22 may be established via any suitable method. In an embodiment, the layers 20, 22 are established via a deposition or manufacturing method. Some non-limitative examples of suitable deposition techniques/manufacturing processes include roll-coating, conventional slot-die processing, blade coating, bent blade coating, rod coating, shear roll coating, slot-die cascade coating, pond coating, curtain coating and/or other comparable methods including those that use circulating and non-circulating coating technologies. In certain instances, spray-coating, immersion-coating, and/or cast-coating techniques may be suitable for depositing.

Further, although the optional coating layer 20 and image-receiving layer 22 are shown in Fig. 2 on both sides 14, 16 of substrate 18 (forming a five-layer system), it is to be understood that the image-receiving layer 22, with or without the coating layer 20, may be on one side 14 or 16 of substrate 18, if desired. In still a further embodiment, the image-receiving layer 22 may be established directly on the substrate 18 on a side 16, 14 opposed the side 14, 16 the layer(s) 20, 22 are established.

It is to be understood that the coating 20, when present, and/or the image-receiving layer 22 may be established at any desirable thickness. In an embodiment, the thickness of each layer 20, 22 ranges from about 5 µm to about 30 µm, and in an alternate embodiment, each layer 20, 22 thickness ranges from about 8 µm to about 15 µm.

The optional base coating 20 and the image-receiving layers 22 may be applied in one or more layers simultaneously, with a coat weight ranging from about 5 g/m² to about 30 g/m², or alternately from about 8 g/m² to about 15 g/m², for each layer 20, 22 on each side 14, 16. In one embodiment, the solid content of the coating colors (i.e. the coating in its liquid state, prior to coating and drying) used to form of each of the layers 20, 22 ranges from about 60 wt% to about 75 wt%. The viscosity of the coating color used to form each layer 20, 22 ranges from about 300 mPas (cps), to about 1500 mPas (cps) as measured by a low shear Brookfield viscometer at a speed of 100 rpm, or from about 30 mP·as (cps) to about 40 mPa·s (cps) at a higher shear rate of 4500 rpm using a high shear Hercules viscometer.

It is to be understood that once the layer(s) 22 (and optionally 20) are established, they may be dried by convection, conduction, infrared radiation, atmospheric exposure. Further, once the layer(s) 22 (and optionally 20) are applied as desired, a calendering process may be used to achieve desired gloss or surface smoothness. The calendering device may be a separate super calendering machine, an on-line soft nip calendering unit, an off-line soft nip calendering machine.

Embodiment(s) of the electrophotographic medium composition 12, 12' and the system 10 include, but are not limited to the following advantages. The composition 12, 12' may be established on a substrate 18 which may be used in high-speed color electrophotographic printing. Without being bound to any theory, it is believed that the one or a combination of the friction control agent(s), substrate 18 stiffness control, and electrostatic charge control via ionic conduction aids, provides a printing media with good running ability in high-speed electrophotographic printing devices over a wide range of environmental conditions.

## Claims

1. A recording medium (10) for electrophotographic printing, the medium (10) comprising:
a substrate (18);
an image-receiving layer (22) established on at least one side (14, 16) of the substrate (18), the image-receiving layer (22) having at least one friction-controlling agent and at least one ionic conduction aid therein; and
a coating layer (20) between the image-receiving layer and the at least one side of the substrate, the coating layer having at least one ionic conduction aid therein;
wherein the medium has a surface resistivity ranging from about 1x10⁹ OHM/square to about 8x10⁹ OHM/square and a volume resistivity ranging from about 1x10⁹ OHM cm to about 5x10¹⁰ OHM cm, at 23°C and 50% relative humidity;
wherein the medium has a stiffness ranging from about 1 Taber unit (0.098066 milliNewton metres) to about 25 Taber units (2.45165 milliNewton metres) in a paper machine direction and from about 1 Taber unit (0.098066 milliNewton metres) to about 15 Taber units (1.47099 milliNewton metres) in a cross machine direction; and
wherein the medium has a sheet-to-sheet static coefficient of friction ranging from about 0.30 to about 0.55, and a sheet-to-sheet kinetic coefficient of friction ranging from about 0.15 to about 0.50, at 23°C and 50% humidity.

2. A medium (10) as claimed in claim 1, wherein a second coating layer (20) is established on a side (16, 14) opposed to the at least one side (14, 16) of the substrate (18), and wherein a second image-receiving layer (22) is established on the second coating (20), thereby forming a five-layer system (10).

3. A medium (10) as claimed in claims 1 or 2, wherein the ionic conduction aid comprises an organic or an inorganic electrolyte, and wherein at least one of the image-receiving layer (22) and the coating layer (20) further includes at least one of inorganic pigments and polymeric binders.

4. A medium as claimed in claim 3, wherein the polymeric binder is a water-dispersible polymeric latex.

5. A medium (10) as claimed in any preceding claim, wherein the medium has a surface resistivity ranging from about 7x10¹² OHM/square to about 1x10¹⁴ OHM/square and a volume resistivity ranging from about 5x10¹³ OHM cm to about 5x10¹⁴ OHM cm, at 15°C and 10% relative humidity.

6. A medium (10) as claimed in any preceding claim, wherein the ionic conduction aid comprises an inorganic or an organic electrolyte, and wherein the electrolyte is at least one of sodium chloride, potassium chloride, sodium sulphate, potassium sulphate, quaternary ammonium salts, polymeric electrolytes, sodium salts of polystyrene sulphonates, ammonium salts of polystyrene sulphonates, sodium salts of polyacrylates, ammonium salts of polyacrylates, sodium salts of polymethacrylates, ammonium salts of polymethacrylates, sodium salts of polyvinyl sulphonates, ammonium salts of polyvinyl sulphonates, sodium salts of polyvinyl phosphates, ammonium salts of polyvinyl phosphates, and combinations thereof.

7. A method of making an electrophotographic medium (10) as claimed in any previous claim, the method comprising:
providing a substrate (18) having two opposed sides (14, 16);
establishing an image-receiving layer (22) on at least one of the two opposed sides (14, 16) of the substrate (18), the image-receiving layer (22) including a friction-controlling agent and an ionic conduction aid, wherein the ionic conduction aid is adapted to substantially control electrical resistivity of the system (10); and
establishing a coating layer (20) between the image-receiving layer and the at least one of the two opposed sides of the substrate, the coating layer (20) having an electrolyte therein.

8. A method as claimed in claim 7, wherein the ionic conduction aid is an electrolyte.

9. A method as claimed in claim 7 or 8, wherein, prior to establishing the coating layer (20) between the image-receiving layer (22) and the at least one of the two opposed sides (14, 16) of the substrate (18), the method further includes mixing the at least one electrolyte with at least one of inorganic pigments and polymeric binders to form the coating layer (20).

10. A method as claimed in claim 7 or 8, wherein, prior to establishing the image-receiving layer (22) on the at least one of the two opposed sides (14, 16) of the substrate (18), the method further includes mixing the friction-controlling agent and the ionic conduction aid with at least one of inorganic pigments and polymeric binders to form the image-receiving layer (22).

11. A method as claimed in any of claims 7 to 10, wherein the establishing is accomplished by blade coating, bent blade coating, rod coating, shear roll coating, curtain coating, slot die coating, pond coating, or cast coating methods.

## Patentansprüche

1. Aufzeichnungsmedium (10) für elektrofotografischen Druck, wobei das Medium (10) Folgendes umfasst:
ein Substrat (18);
eine Bildempfangsschicht (22), die auf mindestens einer Seite (14, 16) des Substrats (18) hergestellt wird, wobei die Bildempfangsschicht (22) mindestens ein Reibungskontrollmittel und mindestens ein Ionenleitungshilfsmittel darin aufweist; und
eine Beschichtungsschicht (20) zwischen der Bildempfangsschicht und der mindestens einen Seite des Substrats, wobei die Beschichtungsschicht mindestens ein Ionenleitungshilfsmittel darin aufweist;
wobei das Medium bei 23 °C und einer relativen Luftfeuchtigkeit von 50 % einen spezifischen Oberflächenwiderstand, der von etwa 1 x 10⁹ Ohm/Quadrat bis etwa 8 x 10⁹ Ohm/Quadrat reicht, und einen spezifischen Durchgangswiderstand, der von etwa 1 x 10⁹ Ohm/cm bis etwa 5 x 10¹⁰ Ohm/cm reicht, hat;
wobei das Medium eine Steifigkeit hat, die von etwa 1 Taber-Einheit (0,098066 Millinewtonmeter) bis etwa 25 Taber-Einheiten (2,45165 Millinewtonmeter) in einer Papiermaschinenrichtung und von etwa 1 Taber-Einheit (0,098066 Millinewtonmeter) bis etwa 15 Taber-Einheiten (1,47099 Millinewtonmeter) in einer Maschinenquerrichtung reicht; und
wobei das Medium bei 23 °C und einer Luftfeuchtigkeit von 50 % einen statischen Reibungskoeffizienten von Blatt zu Blatt, der von etwa 0,30 bis etwa 0,55 reicht, und einen kinetischen Reibungskoeffizienten von Blatt zu Blatt, der von etwa 0,15 bis etwa 0,50 reicht, hat.

2. Medium (10) nach Anspruch 1, wobei eine zweite Beschichtungsschicht (20) auf einer Seite (16, 14) hergestellt wird, die der mindestens einen Seite (14, 16) des Substrats (18) gegenüberliegt, und wobei eine zweite Bildempfangsschicht (22) auf der zweiten Beschichtung (20) hergestellt wird, wodurch ein Fünf-Schichten-System (10) gebildet wird.

3. Medium (10) nach Anspruch 1 oder 2, wobei das Ionenleitungshilfsmittel einen organischen oder einen anorganischen Elektrolyten umfasst und wobei die Bildempfangsschicht (22) und/oder die Beschichtungsschicht (20) weiterhin anorganische Pigmente und/oder polymere Bindemittel enthalten.

4. Medium nach Anspruch 3, wobei es sich bei dem polymeren Bindemittel um einen wasserdispergierbaren polymeren Latex handelt.

5. Medium (10) nach einem der vorhergehenden Ansprüche, wobei das Medium bei 15 °C und einer relativen Luftfeuchtigkeit von 10 % einen spezifischen Oberflächenwiderstand, der von etwa 7 x 10¹² Ohm/Quadrat bis etwa 1 x 10¹⁴ Ohm/Quadrat reicht, und einen spezifischen Durchgangswiderstand, der von etwa 5 x 10¹³ Ohm/cm bis etwa 5 x 10¹⁴ Ohm/cm reicht, hat.

6. Medium (10) nach einem der vorhergehenden Ansprüche, wobei das Ionenleitungshilfsmittel einen organischen oder anorganischen Elektrolyten umfasst und wobei es sich bei dem Elektrolyten um Natriumchlorid, Kaliumchlorid, Natriumsulfat, Kaliumsulfat, quaternäre Ammoniumsalze, polymere Elektrolyte, Natriumsalze von Polystyrolsulfonaten, Ammoniumsalze von Polystyrolsulfonaten, Natriumsalze von Polyacrylaten, Ammoniumsalze von Polyacrylaten, Natriumsalze von Polymethacrylaten, Ammoniumsalze von Polymethacrylaten, Natriumsalze von Polyvinylsulfonaten, Ammoniumsalze von Polyvinylsulfonaten, Natriumsalze von Polyvinylphosphaten, Ammoniumsalze von Polyvinylphosphaten und/oder Kombinationen davon handelt.

7. Verfahren zur Fertigung eines elektrofotografischen Mediums (10) nach einem der vorhergehenden Ansprüche, wobei das Verfahren Folgendes umfasst:
Bereitstellen eines Substrats (18) mit zwei gegenüberliegenden Seiten (14, 16);
Herstellen einer Bildempfangsschicht (22) auf mindestens einer der zwei gegenüberliegenden Seiten (14, 16) des Substrats (18), wobei die Bildempfangsschicht (22) ein Reibungskontrollmittel und ein Ionenleitungshilfsmittel enthält, wobei das Ionenleitungshilfsmittel dazu eingerichtet ist, den spezifischen elektrischen Widerstand des Systems (10) im Wesentlichen zu steuern; und
Herstellen einer Beschichtungsschicht (20) zwischen der Bildempfangsschicht und der mindestens einen der zwei gegenüberliegenden Seiten des Substrats, wobei die Beschichtungsschicht (20) einen Elektrolyt darin aufweist.

8. Verfahren nach Anspruch 7, wobei es sich bei dem Ionenleitungshilfsmittel um einen Elektrolyten handelt.

9. Verfahren nach Anspruch 7 oder 8, wobei das Verfahren vor dem Herstellen der Beschichtungsschicht (20) zwischen der Bildempfangsschicht (22) und der mindestens einen der zwei gegenüberliegenden Seiten (14, 16) des Substrats (18) weiterhin das Mischen des mindestens einen Elektrolyten mit anorganischen Pigmenten und/oder polymeren Bindemitteln beinhaltet, um die Beschichtungsschicht (20) zu bilden.

10. Verfahren nach Anspruch 7 oder 8, wobei das Verfahren vor dem Herstellen der Bildempfangsschicht (22) auf der mindestens einen der zwei gegenüberliegenden Seiten (14, 16) des Substrats (18) weiterhin das Mischen des Reibungskontrollmittels und des Ionenleitungshilfsmittels mit anorganischen Pigmenten und/oder polymeren Bindemitteln beinhaltet, um die Bildempfangsschicht (22) zu bilden.

11. Verfahren nach einem der Ansprüche 7 bis 10, wobei das Herstellen durch Rakelbeschichtungs-, Bent-Blade-Beschichtungs-, Stabbeschichtungs-, Scherwalzenbeschichtungs-, Vorhangbeschichtungs-, Schlitzdüsenbeschichtungs-, Beckenbeschichtungs- oder Gussbeschichtungsverfahren erzielt wird.

## Revendications

1. Support d'enregistrement (10) pour impression électrophotographique, le support (10) comprenant :
- un substrat (18) ;
- une couche (22) de réception d'image, établie sur au moins un côté (14, 16) du substrat (18), la couche (22) de réception d'image ayant au moins un agent de contrôle de frottement et au moins un auxiliaire de conduction ionique dans celle-ci ; et
- une couche de revêtement (20) entre la couche de réception d'image et le au moins un côté du substrat, la couche de revêtement ayant au moins un auxiliaire de conduction ionique dans celle-ci ;
le support ayant une résistivité de surface se situant dans la plage d'environ 1x10⁹ OHM/carré à environ 8x10⁹ OHM/carré et une résistivité volumique se situant dans la plage d'environ 1x10⁹ OHM cm à environ 5x10¹⁰ OHM cm, à 23°C et 50 % d'humidité relative ;
le support ayant une rigidité se situant dans la plage d'environ 1 unité Taber (0,098066 milliNewton mètre) à environ 25 unités Taber (2,45165 milliNewton mètres) dans un sens machine du papier et d'environ 1 unité Taber (0,098066 milliNewton mètre) à environ 15 unités Taber (1,47099 milliNewton mètre) dans un sens travers ; et
le support ayant un coefficient de frottement statique feuille-à-feuille se situant dans la plage d'environ 0,30 à environ 0,55 et un coefficient de frottement cinétique feuille-à-feuille se situant dans la plage d'environ 0,15 à environ 0,50, à 23°C et 50 % d'humidité.

2. Support (10) selon la revendication 1, dans lequel une seconde couche de revêtement (20) est établie sur un côté (16, 14) opposé à l'au moins un côté (14, 16) du substrat (18) et dans lequel une seconde couche de réception d'image (22) est établie sur le second revêtement (20), formant de cette façon un système à cinq couches (10).

3. Support (10) selon l'une des revendications 1 ou 2, dans lequel l'auxiliaire de conduction ionique comprend un électrolyte organique ou inorganique et dans lequel au moins l'une de la couche (22) de réception d'image et de la couche de revêtement (20) comprend en outre au moins l'un parmi les pigments inorganiques et les liants polymères.

4. Support selon la revendication 3, dans lequel le liant polymère est un latex polymère dispersible dans l'eau.

5. Support (10) selon l'une quelconque des revendications précédentes, dans lequel le support a une résistivité de surface se situant dans la plage d'environ 7x10¹² OHM/carré à environ 1x10¹⁴ OHM/carré et une résistivité volumique se situant dans la plage d'environ 5x10¹³ OHM cm à environ 5x10¹⁴ OHM cm, à 15°C et 10 % d'humidité relative.

6. Support (10) selon l'une quelconque des revendications précédentes, dans lequel l'auxiliaire de conduction ionique comprend un électrolyte inorganique ou un électrolyte organique et dans lequel l'électrolyte est au moins l'un parmi le chlorure de sodium, le chlorure de potassium, le sulfate de sodium, le sulfate de potassium, les sels d'ammonium quaternaire, les électrolytes polymères, les sels sodiques de polystyrène sulfonates, les sels d'ammonium de polystyrène sulfonates, les sels sodiques de polyacrylates, les sels d'ammonium de polyacrylates, les sels sodiques de polyméthacrylates, les sels d'ammonium de polyméthacrylates, les sels sodiques de polyvinyl sulfonates, les sels d'ammonium de polyvinyl sulfonates, les sels sodiques de polyvinyl phosphates, les sels d'ammonium de polyvinyl phosphates et leurs combinaisons.

7. Procédé de fabrication d'un support électrophotographique (10) selon l'une quelconque des revendications précédentes, le procédé comprenant :
- se procurer un substrat (18) ayant deux côtés opposés (14, 16) ;
- établir une couche (22) de réception d'image sur au moins l'un des deux côtés opposés (14, 16) du substrat (18), la couche (22) de réception d'image comprenant un agent de contrôle de frottement et un auxiliaire de conduction ionique, l'auxiliaire de conduction ionique étant apte à contrôler sensiblement la résistivité électrique du système (10) ; et
- établir une couche de revêtement (20) entre la couche de réception d'image et le au moins l'un des deux côtés opposés du substrat, la couche de revêtement (20) ayant un électrolyte dans celle-ci.

8. Procédé selon la revendication 7, dans lequel l'auxiliaire de conduction ionique est un électrolyte.

9. Procédé selon l'une des revendications 7 ou 8, dans lequel, avant d'établir la couche de revêtement (20) entre la couche (22) de réception d'image et le au moins l'un des deux côtés opposés (14, 16) du substrat (18), le procédé comprend en outre le mélange du au moins un électrolyte avec au moins l'un parmi les pigments inorganiques et les liants polymères pour former la couche de revêtement (20).

10. Procédé selon l'une des revendications 7 ou 8, dans lequel, avant d'établir la couche (22) de réception d'image sur le au moins l'un des deux côtés opposés (14, 16) du substrat (18), le procédé comprend en outre le mélange de l'agent de contrôle de frottement et de l'auxiliaire de conduction ionique avec au moins l'un parmi les pigments inorganiques et les liants polymères pour former la couche (22) de réception d'image.

11. Procédé selon l'une quelconque des revendications 7 à 10, dans lequel l'établissement est accompli par des procédés de couchage à la lame, de couchage à la lame courbe, de couchage à la barre rotative, de couchage au rouleau de cisaillement, de couchage par voile, de couchage par filière plate, de couchage à la lame de type à cuve ou de couchage au glacis.
